

Patented Sept. 4, 1923.

1,466,747

## UNITED STATES PATENT OFFICE.

PAUL ONNERTZ, OF BERLIN-WILMERSDORF, GERMANY, ASSIGNOR TO ACTIEN GESELLSCHAFT FÜR ANILIN FABRIKATION, OF BERLIN, GERMANY.

### PROCESS FOR DYEING FURS, SKINS, HAIRS, FEATHERS, OR THE LIKE.

No Drawing.

Application filed May 15, 1922. Serial No. 561,011.

To all whom it may concern:

Be it known that I, PAUL ONNERTZ, a citizen of the German Republic, residing at Berlin-Wilmersdorf, Germany (my post-office address being Dusseldorferstr. 72, Berlin-Wilmersdorf, Germany), have invented certain new and useful Improvements in Processes for Dyeing Furs, Skins, Hairs, Feathers, or the like, of which the following is a specification.

It is known to dye furs, feathers, hairs or the like with aid of 4-amino-1-oxybenzene. By my present invention tints which differ considerably from those obtained with 4-amino-1-oxybenzene may be obtained by application of derivatives of 4-amino-1-oxybenzene, containing negative substituents such as halogen-, nitro-group in presence of an oxidizing agent, the shades being of an excellent fastness.

The said derivatives are superior to 4-amino-1-oxybenzene because they may be used mixed with other compounds for example with meta-diamine, whereby dyeings are obtained showing the mixed shades of the components, whereas the unsubstituted 4-amino-1-oxybenzene reacts with many other compounds so that the shades thus obtained differ from those of the components.

The following example illustrates my invention, without limiting it:—

The well-washed skin is handled for some hours at ordinary temperature in a bath which contains per litre 2 grams of 2-chloro-

amino-1-oxybenzene, 4 grams of ammonia (of 25% strength) and 30 cc. of hydrogen peroxide (of about 3% strength). The skin is then well-washed and finished as usual, a brownish shade being obtained.

40 The tints obtained on skins prepared with chromium or copper mordants are brown, those on skins prepared with iron mordants are reddish brown.

2,3-dichlor-4-amino-1-oxybenzene dyes 45 gray tints inclining to green; 2-nitro-4-amino-1-oxybenzene, when dyed on furs prepared with chromium- or copper-mordants, dyes brown shades with a reddish 50 tinge.

Having now particularly described my said invention and the manner in which it may be performed what I claim is—

1. Process of dyeing furs, skins, hairs, feathers and the like, comprising treating the same in the presence of an oxidizing agent with a solution of a 4-amino-1-oxybenzene containing a negative substituent.

55 2. Process of dyeing furs, skins, hairs, feathers and the like, comprising treating the same in the presence of an oxidizing agent with a solution of 2-nitro-4-amino-1-oxybenzene.

60 In testimony whereof I affix my signature in presence of two witnesses.

DR. PAUL ONNERTZ.

Witnesses:

LEO KERKOVIOUS,  
Dr. MAX BRAUNS.